

March 4, 1947.

W. H. FARR

2,416,742

HARROW DISK

Filed Jan. 9, 1943

FIG. 1.



FIG. 2.



INVENTOR  
Warren H. Farr.

BY *John P. Farbox*  
ATTORNEY

## UNITED STATES PATENT OFFICE

2,416,742

## HARROW DISK

Warren H. Farr, Detroit, Mich., assignor to The  
Budd Company, Philadelphia, Pa., a corpora-  
tion of Pennsylvania

Application January 9, 1943, Serial No. 471,851

2 Claims. (Cl. 97—217)

1

This invention relates to harrow disks and particularly to a method and apparatus for heat treating steel disks for harrows and similar uses.

Metal requirements for harrow disks are exacting because of the rough usage to which a harrow is ordinarily subjected. The disk in the usual type harrow must be of metal strong enough to resist curling under the harrow weight; it must resist kinking and nicking due to impact on pebbles or other hard materials; and it should retain its shape and yet possess a certain amount of springiness. Finally, the edge should be able to withstand hard treatment and maintain its cutting qualities.

Carbon and alloy steels are preferable as harrow disk metals, and the heat treatment should be such as to develop the above-mentioned qualities. Frequently, the steel is rolled two ways to develop resistance to bending. Electrical heat treatment lends itself satisfactorily to the securing of appropriate hardness.

Associated with the securing of the desired metal qualities in disk steel, an important object of the invention is to provide a disk having exceptional edge hardness. Another object is to provide a harrow disk having desired yield as a unit combined with overall strength. A further object is the provision of a steel disk highly resistant to curling, kinking or nicking.

An object of the invention also is to provide an improved process for electrically heat treating harrow disks. A further object is to provide a simplified process for securing differential heat treatment on opposite sides of the edge portion of a disk. An object, also, is to provide a process in which the desired edge curvature of the harrow disk is obtained automatically. Additionally, an object of the invention is the provision of simplified quenching means for heated articles.

Further objects relating to the invention will appear on consideration of the following detailed description of the process, apparatus and article, and of the illustrative embodiment of the apparatus and article, such as appears in the accompanying drawing in which:

Figure 1 is a vertical section through the disk and supporting mechanism;

Figure 2 is a plan view of the structure;

Figure 3 is a detail showing the conductor and coolant connections; and

Figure 4 is a detail of the support.

Referring to Figures 1 and 2 of the drawing, there is shown an assembly by means of which the disk 10, as indicated in dotted outline, is sup-

2

ported for heat treatment. Steel disks of the desired type have preferably such a carbon content as to possess, in their normal state prior to heat treatment in accordance with this invention, the measurable degree of yield or springiness under load, associated with toughness, which will afford adequate resistance to impact while in use in various implements, such as harrows. Heat treatment may involve rolling of the metal at different angles so as to distribute the internal stresses with greater uniformity, this being particularly desirable in a disk or wheel subjected to pressure along the entire peripheral edge.

15 The disks 10 are adapted for heat treatment on an inductive heater, generally indicated by the numeral 12, and comprising a single primary coil 14 having spaced integrally and radially projecting lugs 16, extending from the outer surface 20 of the primary coil, and supported on standards 18. The mode of connection between the lugs 16 and standards 18 is clearly shown in Figure 4, a machine screw 20 passing through an eye opening in the lug and having screw-threaded engagement with the top of the standard 18. An insulation sleeve 22 and insulation washers 24 electrically insulate the lug from the standards, these elements being held in position by the bolt washers 26.

30 As indicated in Figure 1, the primary coil is formed of a hollow tube with a square cross-section forming a conduit for cooling liquid for absorption of excess heat developed in the heating process in the primary coil.

35 In Figures 2 and 3, the construction of the primary coil is illustrated as circular with ends 30 in close proximity, the tubular cross-section being closed by means of end plates 32. Conductor terminals 34 and 36 lead from the circular ends 30 of the primary coil, power line connections supplying high-frequency current in excess of 2000 cycles and preferably around 9600 cycles being made to these terminals by means of screw bolts 38, two bolts being utilized for each terminal. As shown in Figure 3, the terminals 34 and 36 are formed with passageways 38 and 40, connecting with the hollow interior of the primary coil 14, and to these passageways pipe connections 42 and 44 are made for the passage 45 of an appropriate coolant through the primary coil.

50 The disk 10 is mounted upon rotatable supporting means centrally positioned within the annular primary coil. These supporting means, indicated generally by the numeral 50, include

a stationary tubular and upstanding frame member 52, the top of which terminates within the levels of the top and bottom planes of the primary coil. Within the tube 52 is positioned a shaft 54 having a reduced upper section 56, which is connected to the tube 52 by means of ball bearings 58 and ball bearing runways 50. A threaded plate 62 normally holds the ball bearing unit in position. Also connected to the reduced upper section 56 of the shaft is a disk-supporting member 64, having a tubular skirt 66 depending therefrom and rotatable therewith. Resting on the flattened top of this member 64 is the disk 10, the end of the shaft 54 being formed with a rectangular section 68, adapted to enter a corresponding central square opening in the disk 10. A holding nut 70, provided with a pin 72 for engagement of a bayonet slot 74, in the top of shaft 54, is adapted for holding the disk 10 in fixed position during the heat treatment process.

Means for quenching the heated disk surface are provided in a plurality of circumferentially arranged, upright and spaced pipes 80, each terminating approximately at the upper plane of the primary coil within said coil, and each being provided with outwardly extending nozzles 82, flattened as shown in Fig. 2 and chamfered angularly so as to direct a broad fan-shaped sheet of liquid quench against the lower peripheral surface of the disk, the same forming an edge annulus. The apparatus as above described may be secured, as by bolts 11, to a circumferential base plate 13, having radial openings 15 spaced from the supporting elements 18.

Having described the essential apparatus for carrying out the process steps of my invention, the operation of the same may now be described in detail.

A flat disk 10, having been appropriately rolled and treated to provide the necessary compression and impact resistance for the central annulus or area of the disk other than the edge annulus hereinabove mentioned, is clamped to the rotatable shaft 54. The shaft is then rotated by any appropriate means with speeds sufficiently high to secure uniformity of heat treatment in the time interval, as required, and to secure the proper control over the quenching liquid, as will now appear. Electrical power is then applied to the primary through the terminals 34 and 36, the coolant in the primary coil being under forced movement, with the result that high-frequency electromagnetic induction is applied to the edge annulus of the disk 10.

As is known in this art, the application of a high-frequency alternating current in inductive relation to a conductor, such as disk 10, induces in the conductor eddy currents variable with frequency, the same constituting a heating means of high effectiveness; due to the skin effect phenomena, heating currents tend to concentrate in the surfaces of the disk, and where the conductor and inductor are closely positioned together, as in the present arrangement, the surface of the disk adjoining the inductor receives a maximum concentration of heat, due to the so-called proximity effect, that is, that effect due to the summation of the inductive effects, by which the reactive magnetic forces at the adjacent surface of the disk 10 are lessened, permitting a larger flow of current and consequent increase in heating action at the adjacent or under surface.

Due to the heating effect which, as described,

results in the concentration of heat on the lower side of the disk, as shown in Figure 1, the disk expands more rapidly on the lower edge annulus, warping the same upwardly and, because of the uniform electrical action around the disk circumference, the warping curvature is substantially uniform. The heat treatment is continued for such a time period that the temperature of the edge annulus 90, as distinguished from the central annulus 92, is above the critical temperature of the material, that is, above the temperature at which molecular rearrangement, due to heat, occurs. It is important that the heat be carried above this critical temperature in order to secure the proper hardness on quenching and further to prevent a subsequent flattening of the disk.

Having heated the disk to the proper temperature for the desired time interval, the electrical power is cut off and the quench immediately applied. There consequently results a contraction of the disk, the contraction concentrating in the edge annulus with a result that a pronounced dishing of the disk occurs, as shown by the disk 94 in Figure 1. Due to the rotation of the disk, the quench liquid is carried to all parts of the heated section of the edge annulus, and the quench is continued until the disk is reduced to ambient temperatures.

In accordance with the described heat treatment, the lower surface 96 of the edge annulus is quenched from a higher temperature than the upper surface 98, and while both surfaces of the edge annulus possess compressional stresses, the stresses on the lower edge 96 exceed those on the upper edge 98. Further, the compressional stresses in the edge annulus 90 are materially in excess of the stresses existing in the central annulus 92. Therefore, on cooling, any tendency to flatten on the part of a disk is resisted, and the disk retains, therefore, a pronounced curvature. If this curvature is not of the desired extent, the heating and quenching may be repeated. Unless the critical temperature of the material is exceeded in the heat treatment, this result usually would not be obtained. As a result of this heat treatment, the completed disk possesses an edge annulus of uniform hardness in conjunction with the more yieldable and tougher central annulus 92, thus making the disk highly adaptable for use in harrows and similar uses.

It is pointed out that through the use of the spout 82 on the quenching pipes 80, the quench liquid is placed directly adjacent the area between the disk edge and the inductor 14, so that considerable pressure can be applied to prevent the formation of steam pockets in this area. Avoidance of steam pockets where water is used is also facilitated by the rotation of the disk as well as by the upward bending of the disk edge to form a flared space for the quenching liquid.

The drawing and description thereof are intended to illustrate an embodiment of the invention which may be preferred. However, modifications of the same may be made such as may come within the scope of the claims hereto appended.

What is claimed is:

1. A dished steel disk having an edge annulus quenched hardened after heating above the critical temperature for steel, the convex annular surface having a hardness greater than that of the concave annular surface.

2. A dished steel disk having an edge annulus quenched hardened after heating above the critical

temperature for steel, the convex annular surface having a hardness greater than the concave annular surface, and a central annulus having lesser hardness and greater flexibility than said edge annulus, the compressional stresses of said convex edge annulus being greater than those of the concave edge annulus.

WARREN H. FARR.

REFERENCES CITED

The following references are of record in the file of this patent:

UNITED STATES PATENTS

| Number    | Name   | Date          | 15 |
|-----------|--------|---------------|----|
| 488,514   | Arnold | Dec. 20, 1892 |    |
| 1,325,770 | Woodin | Dec. 23, 1919 |    |

| Number      | Name        | Date          |
|-------------|-------------|---------------|
| 506,671     | Corbin      | Oct. 17, 1893 |
| 2,254,307   | Mott et al. | Sept. 2, 1941 |
| 1,517,633   | Junkers     | Dec. 2, 1924  |
| 5 2,320,573 | Doelker     | June 10, 1948 |
| 1,959,650   | Verity      | May 22, 1934  |
| 1,711,835   | Davis       | May 7, 1929   |
| 2,280,064   | Denneen     | Apr. 21, 1942 |

FOREIGN PATENTS

| Country  | Date          |
|----------|---------------|
| British  | 1936          |
| British  | July 23, 1937 |
| Austrian | May 30, 1932  |